

# UNITED STATES PATENT OFFICE.

CHARLES CRABTREE, OF NELSONVILLE, OHIO.

## COMPOSITION TO BE USED IN MAKING SQUIBS WATER-PROOF.

SPECIFICATION forming part of Letters Patent No. 242,758, dated June 14, 1881.

Application filed December 23, 1880. (No specimens.)

*To all whom it may concern:*

Be it known that I, CHARLES CRABTREE, a citizen of the United States, residing at Nelsonville, in the county of Athens and State of Ohio, have invented a new and useful Composition of Matter to be Used in Making Squibs Water-Proof, of which the following is a specification.

My compositions consist of the following ingredients, combined in the proportions stated, viz: beeswax, one pound; flowers of sulphur, three pounds; alcohol, one pint; gum-shellac, one-half pound. These ingredients are to be mixed as follows: The beeswax and flowers of sulphur are placed together in a pot over a fire until arrived at boiling-point and are thoroughly mixed. The alcohol and gum-shellac are mixed thoroughly and allowed to stand for twelve hours, when ready for use.

In using the above-named compositions, the squib is first dipped in the composition of beeswax and flowers of sulphur and allowed to dry, this being the first water-proof coat. After the above-named coating is dry the squib is dipped in the composition of alcohol and gum-shellac, which gives it the second water-proof coat, the both compositions used in the manner described making the squib water-proof.

About eight thousand squibs four and two-eighths inches in length by one-eighth inch in diameter can be made water-proof with the quantity mentioned above.

By the use of the above compositions squibs can be made water-proof for at least two hours.

I am aware that Letters Patent were granted S. H. Daddow, December 24, 1872, No. 134,128, wherein is specified that the cheaper class of squibs are made of paper which is varnished with soluble glass or painted with any other fire-proof material; but nothing is specified as to making squibs made of paper water-proof. I have personally given attention and trial of the squibs made of paper under S. H. Daddow's patent, and find they are not water-proof, as they lose their water-proof qualities after remaining five minutes in wet or damp places.

What I claim, and desire to secure by Letters Patent of the United States, is—

The herein-described compositions of matter to be used in making squibs water-proof, one composition consisting of beeswax and flowers of sulphur, the other composition consisting of alcohol and gum-shellac in the proportions specified.

In testimony whereof I affix my signature in presence of two witnesses.

CHARLES CRABTREE.

Witnesses:

CHARLES E. CUTLER,  
HERBEET GRAVES.